

Aug. 21, 1951

J. J. O'CONNOR ET AL

2,565,260

METHOD OF AND APPARATUS FOR COATING PAPER

Original Filed Sept. 26, 1939

5 Sheets-Sheet 1



Fig. 1



Fig. 1A

Inventor

James J. O'Connor  
Russell N. Savage  
Hellmut C. Schewelbe

By

MacEachol and Mac Attorneys

Aug. 21, 1951

J. J. O'CONNOR ET AL

2,565,260

METHOD OF AND APPARATUS FOR COATING PAPER

Original Filed Sept. 26, 1939

5 Sheets-Sheet 2



Aug. 21, 1951

J. J. O'CONNOR ET AL

2,565,260

METHOD OF AND APPARATUS FOR COATING PAPER

Original Filed Sept. 26, 1939

5 Sheets-Sheet 3



Fig. 3

By

Inventor  
James J. O'Connor  
Russell N. Savage  
Hellmuth C. Achimelke

Marshall & Loc Attorneys

Aug. 21, 1951

J. J. O'CONNOR ET AL.

**2,565,260**

## METHOD OF AND APPARATUS FOR COATING PAPER

Original Filed Sept. 26, 1939

5 Sheets-Sheet 4



Fig. 4



Fig. 5

Inventor  
Jones J. O'Connor  
Russell W. Savage  
Hellmuth C. Achibalde  
By  
Macchol Doe  
Attorneys

Aug. 21, 1951

J. J. O'CONNOR ET AL

2,565,260

METHOD OF AND APPARATUS FOR COATING PAPER

Original Filed Sept. 26, 1939

5 Sheets-Sheet 5



Inventor

James J. O'Connor  
Russell H. Savage  
Hellmuth C. Schawalbe

By

Marshall & Nau

Attorneys

## UNITED STATES PATENT OFFICE

2,565,260

METHOD OF AND APPARATUS FOR COATING  
PAPER

James J. O'Connor, Russell H. Savage, and Hellmuth C. Schwalbe, Chillicothe, Ohio, assignors, by mesne assignments, to The Mead Corporation, Chillicothe, Ohio, a corporation of Ohio

Continuation of application Serial No. 296,690, September 26, 1939. This application April 28, 1947, Serial No. 744,294

14 Claims. (Cl. 117—111)

**1** This invention relates to the manufacture of paper, and more particularly paper having suitable application of a finely divided finish imparting mineral to the surface thereof to provide a printing surface adaptable for high grade and exacting printing requirements, such as half-tone and multiple color reproduction work in magazine illustrations and the like, and is adaptable for use in the manufacture of such paper as a continuous paper making operation.

One of the principal objects of the invention is to provide a new process of producing such paper with a mineral finished surface of high degree of smoothness and finish adapting it for such high grade multi-color reproduction and half-tone magazine illustration work, and with high speed operation to produce a product of quality equal to, or comparable with, that of mineral finished or coated paper as made by any other practiced process which is efficient and effective in operation and its controls.

Another object is to provide a process for producing a mineral suspension which may be effectively and efficiently applied to produce such a paper having said quality surface finish.

Another object is to provide a process of applying such mineral material to paper to produce paper having such surface finish.

Another object of the invention is to provide novel apparatus for carrying such processes into effect to produce such products.

Still another object of the invention is to provide novel apparatus, adaptable for use in the manufacture of a book paper having a mineral finished surface of the characteristics described as a continuous paper making operation and applied under varying degrees of moisture content of the formed paper web, and providing for unusual effectiveness in the production of such paper.

Other objects and advantages of the invention will be apparent from the following description and claims and the drawing, when considered in connection each with the other.

In the drawing, in which like characters of reference designate like parts throughout the several views thereof.

Fig. 1 is a diagrammatic view in side elevation of the first section of a paper making machine constructed according to, and for carrying out, the preferred embodiment of the invention;

Fig. 1A is a corresponding diagrammatic side elevational view of the remaining portion of said machine, the line A—A, which appears at the right and the left ends of Figs. 1 and 1A respec-

tively, indicating the line of division between these two portions of the continuous machine, for purposes of illustration herein;

Fig. 2 is an enlarged side elevational view of one of the units for applying the final surfacing mineral suspension to the paper web;

Fig. 3 is a view in elevation, with some parts in section and other parts omitted for clearer illustration, at right angles to Fig. 2, along the line 3—3 of Fig. 2 and looking in the direction of the arrows, and with parts omitted for clearer illustration;

Fig. 4 is a detailed view of parts of the mechanisms of Fig. 2;

Fig. 5 is a corresponding detail view of the same mechanisms, shown at right angles to Fig. 4;

Fig. 6 is a diagrammatic view of the apparatus for preparing and treating the mineral surfacing suspension and for supplying it to the final mineral surfacing units; and

Fig. 7 is a diagrammatic, detailed, view in end elevation of an alternative arrangement of color metering rolls.

25 This application is a continuation of our pending application S. N. 296,690, filed September 26, 1939, and now abandoned.

It has been well recognized for many years in the paper industry that the printing characteristics of a paper sheet may be improved by proper surface application of a finely divided mineral suspension, usually known as "coating color," to the surface of the sheet. For many years so-called coated paper has been made and used, particularly in the more exacting types of printing such as multiple color reproduction and half-tone work for magazine illustrations and the like. For many years the most usual commercial practice, so far as known to us, was to apply a suspension of mineral and adhesive in water to the surface of a sized paper and to utilize suitable brushes to spread this suspension to provide a uniform and properly smooth film. In such operations it was the practice to utilize a comparatively hard sized paper and a coating color of comparatively low solids content and therefore very fluid because of its large quantity of water so that when applied to the water-resistant sized surface the brushes could act to cause the material to spread to provide a uniform smooth covering film.

Some years ago applicants' original assignee evolved and has made large commercial use of methods of, and apparatus for, coating paper webs, of varying weights, involving the use of

metallic spreading rolls or knife edge members arranged to provide relative movement with reference to the direction of travel of the paper and to act upon the mineral suspension on the traveling web so as to smooth and spread the mineral material adequately and produce a comparable high grade mineral surfaced sheet, and in which the coating colors were of higher solids content than formerly used and higher solids speeds could be attained.

Likewise, applicants' original assignee, subsequently developed methods of and apparatuses for manufacturing and treating paper whereby mineral color suspension could be applied in and upon the surface of the traveling formed web to give a surface impregnation or a composite impregnation and light-weight coat, or a coat applied upon the surface in desired quantity, for the desired mineral finished surfacing.

Likewise use was made in the paper making industry of a printing press mechanism having usual ink rolls, operated so that the mineral pigmented color suspension, with greater solids consistency than ordinarily used in the coated paper industry under the other processes as described, as in printing would be passed through such spreading ink rollers, such as used for working and spreading ink into a suitably uniform and preworked film for transfer as such to the paper, whereby to work and spread the pigmented suspension into a preworked continuous film of the proper low water content and characteristics to be delivered finally upon the printing roller which would transfer it to the surface of the paper sheet as a continuous preworked printed film.

According to the present invention a mineral surfaced paper product may be produced having a desired quantity of mineral material, up to comparatively large amounts, applied to and spread uniformly upon the surface of the sheet, at very high paper making speeds, to provide a product of superior appearance and printing characteristics equal to or comparable with the best products made by the other processes and yet economically produced.

In the form of apparatus shown, which diagrammatically illustrates a preferred form of apparatus used satisfactorily in operations on commercial scale, a suitable paper stock is supplied to the head box, or other form of inlet 10, for supplying the fibrous stock or furnish to the fourdrinier, or other forming wire, which is indicated by the numeral 11, and passes over the breast roll 12 and the couch roll 13, which is preferably of the suction couch type. The formed paper web is then transferred to a felt 15 for the first roll 16 of a multiple roll press, the web passing over that roll on the felt through the first nip, around the bottom of the second roll 17 to be picked up again at the second nip and passed with a felt over the third roll 18 after which it is picked off of the felt 19 and passed through the rolls of a smoothing press indicated by the numeral 20. As the practicing of the present invention makes it desirable to control in a predetermined manner the surface finish and smoothness of the paper web and also the uniformity of formation, porosity, receptivity and absorptivity thereof for the fluent constituents of the mineral suspension thereafter applied to it, and its inherent and maintained resiliency, with respect to the subsequent operations to which it is subjected, the formation of the paper itself is controlled accordingly beginning with selection

of the stock or furnish from which the web is formed.

Very satisfactory operations under commercial conditions to produce a very satisfactory and high grade finished product has been secured using a raw stock furnish comprising—

| 10 |                 | Aver- | Range |      |
|----|-----------------|-------|-------|------|
|    |                 |       | Low   | High |
|    | Soda.....       | 45    | 30    | 60   |
|    | Sulphite.....   | 15    | 0     | 35   |
|    | Groundwood..... | 10    | 5     | 20   |
|    | Broke.....      | 20    | 15    | 40   |
|    | Kraft.....      | 10    | 0     | 30   |

Material variations are permissible depending upon the subsequent pressures, constituents, consistency, freeness and flowability of the color, paper speed, etc. The soda, sulfite, and groundwood stocks are terms well known and understood in the paper industry, such forms of pulp being generally used throughout the industry to manufacture webs of paper in which one or both surfaces are subsequently treated with mineral suspensions to produce what has been generally known and widely used for many years as surface treated or coated paper; and the term broke is likewise well understood in the paper industry to designate the commercially unusable paper which is produced in paper manufacturing as a result of breaks in the web at which time many hundreds of feet of paper may be run off by the paper machine before the operators can stop the machine and rethread it and resume the manufacture of the regular commercial paper. The broke of course contains the same amounts of the several constituent pulps and other materials as the commercial paper, and when broke is used the paper manufacturer knowing the relative proportions of the several kinds of pulp and other constituents therein can readily determine the actual quantity of each of the several constituents which is being added. Of course, where the broke is re-used in the manufacture of paper from a furnish of the same constituents as is contained in the broke itself, the production problem of determining the amount of broke to add is simple, and in operation skilled production men in the paper mill can and do figure the relative constituents of the furnish for any particular paper to be manufactured as part of their everyday job.

As we have found that the upper or so-called felt side of the web may have pits and irregularities which in magnitude and depth greatly exceed any irregularities and coarseness of interstices present on the wire side of the web, this undesirable condition is diminished by selecting a raw stock furnish of pulps chosen to give uniformity of formation, to have controlled freeness, and by thus and through operation of the paper machine controlling the escape of water during the web formation to produce the desired uniformity and to diminish the magnitude, frequency and depth of the pits or craters which are usually present in the top or felt side of a formed sheet. This desired uniformity and smoothness of formation may be facilitated by delaying the rate of water escape during the earlier stages of formation. Also the dandy roll 21 should be located to operate at such degree of wetness of the formed web as to add to the desired unusual smoothness or lack of craters in the felt side without adversely affecting the internal forma-

tion, the porosity and absorptivity and receptivity of the sheet; and the pressure at the smoothing press 20 should be correspondingly controlled to that same end.

From the smoothing press the paper web which is indicated by 25 passes through a drier section, of usual construction and comprising a suitable plurality of drier rolls 27, with the drier felts 28 and supporting rolls, drive, etc.

After the paper has been suitably dried, according to its inherent characteristics and the subsequent processing, it is subjected to a compacting and smoothing operation. This may be accomplished by the utilization of the calender 30 or the calender 31, or both together in balanced operating relationship.

As illustrated the calender 30 is a two roll calender, and is located between two sections of drier rolls in such position in the drier section that the sheet will have been dried to a moisture content of substantially 35% or lower, and satisfactorily down to a moisture content as low as of the order of 10%. This calender has its pressure adjusted with respect to the moisture content of the web, its formation, inherent resiliency and subsequent processing. Generally speaking the required calender pressure varies with the moisture content of the web; and for a given web the higher the moisture content the more readily the paper web responds to this treatment, i. e. the pressures required vary inversely as the moisture content. Care must be taken to limit the amount of pressure with respect to the character of the web and to control its uniform application for a substantially uniformly formed web to avoid crushing the paper unduly and irregularly. The calender operation should be controlled to compact the paper to such extent as will leave it capable of withstanding any subsequent calendering pressures of the process without the danger of objectionable subsequent crushing of the paper and the mineral upon its surface to disrupt the continuity thereof. Also the calendering operation is conducted so as to smooth out the surfaces, especially to sufficiently diminish the irregularities and pits of the felt side and to bring all those irregularities within the dimensions and quantitative limits of the suspension subsequently to be applied. That is, the traveling paper web is subjected to a controlled rolling operation, under pressures such that proper smoothing of the surfaces will be accomplished and likewise the web will be compacted throughout its extent, from surface to surface, so that with the moisture content of the web and its character and formation properly coordinated with the rolling pressures, there will be such breaking down of looseness of formation throughout the body of the web as will give the desired uniformity of formation, absorbency, etc., with a predetermined retained consolidation or compacting but with treatment such that the inherent resiliency of the web will not be exceeded. That is, while the rolling pressure effective upon the web will tend to smooth out any surface irregularities in the web and will also compact the body of the web, thus decreasing its thickness or caliper to some extent; nevertheless, the rolling pressure is controlled and coordinated with respect to the moisture content, and the character of formation of the web so that while its surfaces are properly smoothed and the body of the web compacted throughout prior to the application of the mineral suspension, nevertheless such compacting does not exceed the inherent resiliency of the fibrous structure of the web so as to de-

stroy that fibrous structure and therefore the compacting is not so conducted as to completely exceed the inherent resiliency of the web and the smoothed and compacted web while thus of lesser thickness or caliper and having smoother surfaces nevertheless has retained its springy or resilient characteristics and when the rolling pressure is removed it will be capable of predetermined limited amount of increase in thickness as it leaves the nip of the rolls causing rolling pressure, and therefore the action is one which has been termed reversible compacting with the inherent resiliency of the web retained, rather than a compacting which is carried to such extent that the inherent resiliency is exceeded and the web crushed and left so that the compacting action at the nip of the rolls giving such rolling pressure is irreversible and the web crushed and broken down because of its inherent resiliency having been exceeded.

The other calender 31 is shown located at a position where the moisture content of the paper, with the number of drier cylinders shown, would be not in excess of 10% and, with such character 25 of raw stock furnished as described above satisfactorily, and even preferably, as low as 3% to 5% or 6%. Since the paper web at this considerably reduced moisture content range has an inherent resiliency and resistance to deformation which is considerably greater than with the moisture content range indicated for the location of the calender 30, and also greater forces are required for effecting required smoothness of surface irregularities to substantially within the 30 range of thickness and quantitative limits of the later applied color suspension, it will normally require substantially greater pressures and also a larger number of calender rolls and nips, our experience in practicing the present invention having indicated that a calender, as described herein, 35 having usual metal rolls and using five nips and two or three weights on the lever arms, will be satisfactory with the paper web as made from the above described furnish and with moisture content of from 3% to 6% or 3% to 8%. Both calenders 30—31 need not be provided; but with both available greater flexibility in operation to meet a wider range of conditions is provided. Each calender is constructed in the usual way so that varying pressures may be exerted at the nips and so that, when desired, rolls may be opened 40 to be non-operative on the paper. Thus either or both of the calenders may be used as desired and the paper web treated under the conditions of moisture, etc. to give most favorable results of compacting, smoothing, etc. In actual commercial operating conditions under conditions such as described above satisfactory results have been secured when operating to produce a coated book 45 paper when using the calender 30 with the nip pressure of the order of 135 pounds per linear inch; and when using the calender 31 with nip pressures of the order of 320-350 pounds per linear inch. The operating tolerances in the calender 30 are closer than with the calender 31.

Having been properly compacted and smoothed to give the desired surface free from objectionably obstructing pits, ridges or crevasses, the paper web is then passed to the nip of a pair of rolls, shown diagrammatically in Figs. 1-1A and Fig. 6, and more in detail in Figs. 2-5. The upper of these rolls is indicated by the numeral 50 35 and the lower by the numeral 36, and which are shown in greater detail in Figs. 2 and 3. Each of these rolls as shown has a metal core

and a rubber surface layer. The rolls are alike except for surface hardness, and the rolls in the machine illustrated and satisfactorily used in operation are approximately 30 inches in diameter—the top roll having a rubber cover of 1 P. & J. hardness and the bottom roll a rubber cover of 35 P. & J. when measured with a  $\frac{1}{8}$  inch ball. The term "P. & J. hardness" is one which is well known in industry, such as the paper industry, which uses rubber covered rolls and is in common usage to indicate the hardness or softness of the rubber layer covering such a roll; and in the paper industry and other industries, it is common practice to order from rubber manufacturers rolls which are rubber covered by designating the character of the roll in terms of the P. & J. number, that number having been fixed by the rubber roll manufacturers themselves and having a well known meaning. Generally speaking, the P. & J. numbers involve the amount of depression made by a one-eighth inch steel ball in the surface of the rubber under a kilogram weight, measured in hundredths of a millimeter. It is usually measured by an instrument developed by the Pusey and Jones Company which is used for the calibration of the hardness or density of rubber covering for rolls. The rolls are so constructed that the cores carrying the rubber surfaces are of extreme rigidity to prevent objectionable sagging or with suitable crowning to compensate therefor; and satisfactory results have likewise been attained using one roll, preferably the upper, having a chromium plated metal surface and the other roll a rubber surface of the character described for the bottom roll. Also under proper conditions the rolls may be reversely positioned with the hard surfaced one below and the softer one above.

Each of these rolls 35 and 36 turns so that its surface travels in the same direction as the paper, and they have associated with them metering rolls which function accurately to meter onto the surface of each of the rolls 35-36, beyond its respective metering roll, a predetermined and accurately controlled quantity of mineral suspension, so that an accurately controlled quantity of such suspension is carried on the surface of the roll into the nip between these rolls 35 and 36, where the traveling paper web enters the nip to pass between these two rolls 35-36. As shown more particularly in Fig. 2 the paper web 25 is illustrated as entering the calender 31, the rolls of which are supported in usual manner in a framework 40, the web 25 passing from the calender, in direction indicated by the arrow, and traveling then to pass between the nip of the rolls 35-36.

As illustrated more in detail in Figs. 2, 3, 4 and 5 the framework 40 has attached to it the overhead frame member 45, the opposite end of which is supported on the standard 46. There are two of these beams 45, as shown in Fig. 3, with a cross beam 47 supported between them, and generally located to be somewhat above the rolls 35 and 36 for supporting part of the adjusting and moving mechanism hereinafter referred to. Fastened to the standard 46, midway of its height is an overhanging extension or bracket 48, which has connected to it by a suitable bearing indicated by the numeral 49, a pivoted supporting arm or member 50.

As shown in Fig. 3 there are likewise two of these pivoted arms 50, each of which has attached to it a depending bracket 51, which in-

cludes a bearing for one end of the shaft 57, of the roll 35.

Mounted upon the floor are two standards or support members 55 each of which carries an upwardly extending bracket 56, likewise having a bearing for supporting one end of the shaft 58 of the roll 36.

The pivoted arm 50 is provided with suitable moving and pressure controlling mechanism whereby the roll 35 may be moved to or from the roll 36 so as to position them against each other with the necessary and predetermined pressure for the particular operating conditions present at the nip for the character of the paper web passing therebetween, the other conditions of the color, etc., and for the final product desired. For effecting such movement and adjustment of the member 50, and the rolls 35 and 36 with respect to each other, each member 50 has pivotally attached to it an arm or connecting rod 60, illustrated as a pair of such connecting rods for each member 50, each of the pair attached to one side of its cooperating member 50. The upper end of each pair of the members 60 is pivotally connected to a crosshead 61. Each crosshead 61 has slidably positioned therein a shaft 62, having a collar 63 on the upper end thereof above the crosshead and another collar 64 thereon below the crosshead. A spring 65 is positioned around each of these shafts between the crosshead 61 and the upper collar 63 and a spring 66 between the crosshead 61 and the lower collar 64. A motor 67 is mounted upon one of the beams 45, which drives through a suitable reduction gearing indicated generally by the numeral 68, to the cross shaft 69, which in turn is in driving connection at its opposite ends with the oppositely positioned shafts 62 so that upon actuation of the motor the shaft 69 will be rotated to cause movement of each shaft 62 against the action of the respective springs 65 and 66, to urge the roll 35 against the roll 36 with a predetermined selected pressure, or to lift the roll under spring pressure against the weight of the roll and its supporting parts to give a nip pressure between these rolls less than that which would normally be furnished by the weight of the roll and its parts. 69' indicates a hand wheel which is mounted on the shaft 69, at the end opposite from the motor, and which can be used alternatively for manual operation as described.

A spring pressed slip clutch, indicated generally by the numeral 70 is provided between the motor and the cross shaft 69 to avoid pressure shocks in operation. Also the crosshead 61 carries two pressure indicator devices each comprising a sector and an indicating finger movable with respect thereto, the sector 75 and cooperating finger 76, which is connected by means of a flexible connection to the lower collar 64 serving to indicate the downward pressure exerted at the nip of the rolls 35-36, this indicating mechanism being actually responsive to the spring compression, but calibrated to read directly the nip pressures. Inasmuch as the lower spring 66 serves, in operation, to exert a lifting force tending to rotate the member 50 about its pivot against the weight of the roll 35 and its connected parts, the member 75 is calibrated to read directly the nip pressure in terms of the weight of the parts which is thus unbalanced and effective to exert a nip pressure between the rolls. In the actual machine illustrated the weight of the upper roll parts gives a turning movement exerting 312 pounds per linear inch as a maximum and the

member 75 is thus calibrated up to that pressure.

Likewise the upper collar 63 has a flexible connection with the indicating finger 77 which is pivoted upon the crosshead and cooperates with a calibrated sector 78, this mechanism being calibrated for indicating directly the nip pressure between the rolls 35 and 36 resulting from actuation of the motor 67 to apply a turning force to the arm 50, in addition to the turning force developed by the weight of the parts, as heretofore described. As the pressure thus exerted supplements that indicated at 75' the member 78 is calibrated to read pressures from 260-460 pounds per linear inch up. By means of this arrangement extreme nicety of pressure control at the nip is attained.

Pivotedly mounted upon each member 50 is an arm 85, the lower end of each arm carrying a bearing to support one end of the shaft of the metering roll 37. The upper end of each member 85 is pivotally connected to a crosshead 86, which is in turn connected to an adjusting shaft 87, having a collar 88 carried thereby, with a spring 89 surrounding the shaft 87 and located between the crosshead 86 and the collar 88.

Rotatably mounted in a pair of upward extensions, one carried by each of the pivoted members 50, is a cross shaft 90, the end of which is shown by the numeral 90 in Figs. 2 and 5. This shaft, at each of its opposite ends, is operatively connected to one end of one of the shafts 81, so that it may be oscillated or swung in opposite directions and, for example, when moved in one direction it will act through the collar 88 to compress the spring 89 against the crosshead 86 and thus swing the pivoted arm 85 to urge the metering roll 37 against the surface of the roll 35, with a force determined by the operating pressure thus exerted and when moved in the opposite direction will tend to lessen the pressure of the metering roll against the roll 35. In Fig. 3 the location of this upper metering roll 37 is indicated in dotted lines. At one end the shaft 90 is connected by means of a universal joint 91 to an impeller shaft 92 which in turn is connected through another universal joint 91' and a slip clutch 93, which is driven by the motor 94, suitable speed reduction gearing being interposed between the motor and the friction clutch, as indicated at 95. This assembly of motor and impeller shaft, etc., is suitably supported by being suspended from the beam 41', which is extended in line with the cross beam 41, one end of it being supported upon one of the members 45 and the other end being supported in any suitable way—as by means of a bracket mounted upon the building wall, or the like.

The member 88 has attached to it a pressure indicating mechanism comprising a calibrated sector member 96, having a cooperating indicating finger 97, the finger 97 being connected by a flexible member to the relatively stationary crosshead or pivoted arms 85, this construction in effect making the finger 97 movable in direct response to flexure of the spring 89, and a spring 98 being attached to the finger 97 to urge it in the opposite direction, as a restoring spring. This sector 96 is calibrated to indicate directly the pounds pressure at the nip between the contacting rolls, in terms of nip pressures per linear inch, as is the case also with the indicating mechanisms heretofore described; and as the roll 37, as indicated, is preferably mounted so that there is substantially negligible turning mo-

ment due to the weight of the parts, very accurate direct pressure adjustments can be made with comparatively simple mechanism—pressures accurate to the unheard of nicety in paper machine roll adjustments of not to exceed 4 pounds per linear inch.

As described, the roll 37 is independently adjustable through the pivoted arm 85 to give the desired nip pressure with respect to the roll 35, and without disturbing in any way the setting or adjustment of the roll 35 with respect to the roll 36. Furthermore, the construction is such that the member 50 may be swung about its pivotal mounting to control the nip pressure between the rolls 35 and 36, or to swing the roll 35 entirely away from operative relation with the roll 36 for purposes of clean up, repair to the rolls or the like. This is particularly advantageous in that the rolls 35 and 36 may be thus relatively adjusted to take care of varying weights of the paper and other operating variations without the necessity of changing the metering roll adjustment from a satisfactorily operating condition. It is in order to accomplish this that the universal joint construction of the impeller shaft 92 is provided, this construction permitting relative adjustment of the metering roll with respect to the roll 35 with proper driving of the cross shaft and without disturbing setting if the member 50 is moved about its pivots.

The paper web 25 passing from the calender is preferably passed over a cooled roll 110, which is freely rotatable in bearings mounted upon springs, illustrated diagrammatically at 111 in Fig. 2 and maintained under suitable tension range coordinated with the tension of the web of paper as it passes from the calender into the nip of the mineral suspension applying rolls 35-36. This roll is cooled in order to make sure that the residual temperature of the paper web as it comes from the drier cylinders is not excessive, as it goes into the color application zone. Another roll 112 is positioned just in advance of the inlet of the nip between the rolls 35 and 36 for controlling the angle of approach of the web being processed as it passes into the nip, this roll being likewise suitably mounted for free turning with the paper, in suitable bearings.

In order to provide a proper amount of mineral suspension to be applied to and upon the surface of the traveling web such prepared mineral suspension is fed into the nip space between the rolls 35 and 37, which space acts as a trough to receive and contain a supply or pond of mineral suspension. Inasmuch as the amount of mineral supplied to the paper web should be accurately controlled for desired operating conditions to produce a desired end product, it is preferable to maintain a substantially constant depth in the pond of mineral suspension, entirely across the length of the rolls. Furthermore, it is desirable to maintain the pond of mineral suspension or color substantially uniform in its characteristics clear across and thus to prevent irregularities and undesirable variations in operation which might otherwise result. In order to maintain the predetermined and uniform head in the pond, and also to supply the mineral suspension thereto so as to maintain uniformity of composition and characteristics clear across, means is provided for supplying the mineral suspension through a plurality of pipes or nozzles, which are oscillated back and forth across the face of the rolls, so as to continuously replenish the mineral suspension in the pond throughout its entire transverse extent. Mechanism for accomplishing this is

11

shown more in detail in Figs. 2, 4 and 5. The prepared mineral suspension of desired composition and characteristics is pumped to a manifold 115, properly supported from the members 45. As shown, one end of this manifold is connected by the delivery pipe 25 to the discharge end of the pump whereby the mineral suspension is transferred from the machine storage tank or chest 240 (see Fig. 6 and description below), the other end being open for discharge of any excess back to the machine storage chest through the return pipe 263, the construction and operation being such that an excess of the color is pumped to and through this manifold 115. A plurality of pipes 116, each having a control valve 117, open out of this manifold 115, the manifold 115, and the depending pipes 116, being located substantially above the nip-trough between the rolls 35-37. By means of the individual control valves 117 the amount of suspension fed through each pipe may be accurately controlled to attain the desired conditions of feed into and within the nip-trough. The lower end of each pipe 116 has a flexible tube 118 attached thereto, which in turn carries at its lower end a nozzle or pipe 119. As a means for effecting desired movement of these nozzles they are shown as passed through a plate 120 the opposite ends of which are pivotally connected to depending straps 121, the upper end of each strap being also pivotally connected to a bracket 122 attached to the stationary supporting framework heretofore described. One of the members 50 has attached to it an upstanding bracket 123, carrying a rotatable pulley 124 having a crank arm 125 which is connected by means of the rod 126 to one of the straps 121 so that upon rotation of the pulley 124 oscillating motion will be imparted to the rod 126 to oscillate the plate 120 in a direction parallel to the axis of rotation of the two rolls 35 and 37 and longitudinally of the nip-trough. In the construction shown an oscillation of approximately 6 inches to each side is imparted to the nozzles 119 and the nozzles themselves are therefore positioned apart a distance slightly in excess of 12 inches, substantially the same as the full stroke movement of the nozzles. The pulley 124 is connected by means of a belt 127 to a driving pulley mounted upon the shaft 129, which in turn is supported in a second bracket 128, which shaft also carries a driven pulley 129', connected by means of a belt 130 to one end of the shaft of the roll 36, as shown in Figs. 4 and 5. By means of this construction the plate 120 is oscillated in timed relationship with respect to the rate of rotation of the roll 35, and as the roll 37 is controlled to rotate in predetermined speed relation with the roll 35, the result is to feed the mineral suspension into the nip-trough in a relationship controlled with respect to the rate of operation of the rolls 35 and 37. This, in conjunction with the adjustment of the several valves 117 will give a predetermined feed of the mineral suspension, will maintain predetermined head completely across the nip-trough, and will prevent the segregation of any of the color suspension as a result of forming dead pockets so that the color in the nip-trough will be of substantially uniform composition and characteristics throughout any instant of operation, and thus by proper preparation, processing and control in handling may be maintained of predetermined, substantially constant controlled composition and characteristics for long operating periods with respect to the character, receptivity,

12

absorptivity, etc. of the web and the end product; or varied in controlled and selected or predetermined manner and extent as desired. The color suspension has been previously admixed into thorough uniformity and in the apparatus shown for delivering the maintained quantity to the nip-trough for working and metering need be only sufficiently fluent to be pumped to the nip-trough.

The lower roll 36 is provided with a similar, and similarly operating, metering roll. The desired operating effect of this metering roll is the same as that of the metering roll 37, as described above. And in Fig. 7 a fragmentary view, the lower color application roll, designated in this view by the numeral 36a, has associated with it a single metering roll 37a, having the same sort of operating and pressure adjusting mechanism described above with respect to the other metering roll 37, (and therefore not shown in this view) to vary the setting thereof with respect to its color application roll 36a. However, in the operating machine which is illustrated in the drawing for example in Figs. 1 through 5, the arrangement and location of the machine is such that greater effectiveness of the operators in practical operation of the machine and increased safety conditions are secured with the metering roll for the lower roll 36 placed upon the opposite side or paper web inlet side, as illustrated in Fig. 2. Therefore the adjusting mechanism for the roll 37a is not illustrated, and the preferred operating construction is illustrated in Fig. 2 and described in connection therewith. It is sufficient, with respect to the form of construction somewhat diagrammatically illustrated in Fig. 7, to state that the roll 37a is the same in its construction, adjustment and operation with respect to metering as the roll 37 which may be attained by obvious rearrangement of the supporting, driving and adjustment mechanism herein specifically described. As is indicated by direction indicating arrows, the surface of the roll 36a in juxtaposition to the metering roll 37a is turning downward, and consequently the surface of the metering roll 37a turns in the same direction. And this arrangement provides a nip-trough, available to receive the color suspension through the manifold 115' and connected feed pipes, the whole mechanism being arranged to give the same control of the color suspension in the nip-trough, the accurately controlled metering, etc., as described above. For purposes of simplicity of disclosure in the drawings, this means for supplying the color suspension to the nip-trough, for the lower rolls, is illustrated more or less diagrammatically, it being understood that the more desirable feature to be preserved is the supplying of the color to this nip-trough so as to cause substantially uniform head and substantial uniformity throughout the extent of the nip-trough. In this diagrammatic illustration the flexible tubes and the oscillating arms and plates for causing movement thereof are not shown; but the manifold 115' is shown diagrammatically, in practice being supported by any suitable mechanism so that it may be oscillated back and forth. This mechanism is not specifically illustrated or described in all details, since its construction and operation are the same as the correspondingly numbered parts as illustrated in detail in Figs. 3, 4 and 5 in connection with the manifold 115 and associated parts and fully described in connection therewith. For effecting this oscillation a projecting member is

attached to the manifold, which in turn receives one end of an oscillating connecting member 126' (see Fig. 2) which in turn can be driven by mechanism such as that shown in Fig. 4, and described elsewhere as stated. This mechanism would impart proper oscillation to that portion of the manifold which directly serves the nip-trough for the lower rolls, and suitable flexible connection would be interposed between the two portions of the manifold to permit this.

As shown in Fig. 2, however, the surface of the roll 35 contacting with the surface of the metering roll 37' is traveling in an upward direction and consequently the surface of the metering roll travels likewise. On this account the space above and between the two rolls is the discharge space of the metering nip instead of the inlet space in contrast with the other two conditions described. In order to provide for maintaining the same uniform and accurately controlled composition and characteristics of the color suspension to be metered onto the surface of the roll 36, a second roll 140 is provided and so mounted that it may be pressed against the roll 37' as desired.

Supported upon the standard or supporting member 55, at each side of the machine, by a suitable pivot bearing 141, is a roll supporting member 142. Each of these members has attached to it an upstanding extension 143 which carries a bearing for the corresponding end of the shaft of the metering roll 37'. Each member 142 likewise carries an extension 144 which is pivotally connected to the member 142 by means of a pivot bearing 145, each such upwardly extending pivoted member 144 carrying a bearing for one end of the shaft of the roll 140. The pivoted member 142 also carries a lower extension which is connected by means of a pivot 146, to an adjusting shaft, which is surrounded by a spring located between two collars, these parts being enclosed within a housing 147. This mechanism is likewise operated by a suitable motor and gear reduction indicated generally by the numeral 148, driving cross shaft 148' (see Fig. 3); and has pressure indicating mechanism indicated generally by the numeral 149 and calibrated to indicate directly the pressure conditions at the nip of the rolls 36 and 37', the construction and operation of such part being as described above in connection with rolls 37 and 35.

Pivotedly attached to the upper end of the extension 143 is a shaft or rod 150, the opposite end of which carries a hand wheel 151, which, upon rotation, actuates the spring containing cylinder 152 to move it axially of the rod 150. The cylinder 152 is a cup shaped member with one end of the spring resting against a bottom or suitable internal flange therein, the other end of the spring resting against a collar 153 carried by the rod 150. The cup shaped member floats on the rod 150 and has a knife-edged type of pivot member indicated at 154 to be located within a corresponding notch in the cooperating face of the upward extension 144 which supports the roll 140. By turning the hand wheel 151 pressure is exerted upon the spring and transmitted to the cup member and its pivots 154 to press against the extension 144 and swing that extension about its pivot 145 to urge the roll 140 toward to roll 37' under the desired tension pressure of the spring. Means for feeding the color suspension to the nip-trough between the rolls 149 and 37', and maintaining a desired predetermined head and uniformity of composition and characteristics of distribution of the color within the

nip-trough is provided which means is substantially a duplicate of the means described above, the color supplying manifold being indicated by the numeral 115, the flexible pipes 118' for permitting oscillation of the nozzles 119', and the other parts corresponding.

As is the case with the mechanism described in connection with the upper roll the pivoted member 142 carries both rolls 37' and 140 so that the parts may be moved as a unit about the pivot 141 to vary the position of the metering roll with respect to the color application roll 36 without disturbing the relative setting of the rolls 37' and 140; and likewise the roll 140 may be given independent adjustment without effecting the setting at the metering nip.

The color supply maintained in the nip-trough is carefully controlled with respect to its solids content, its adhesion-tension for the surfaces of the rolls 35-36 and also for the paper web, its freeness, the receptivity of the sheet for the mineral suspension and the various constituents thereof, its consistency, its thixotropic characteristics, etc., so that in operation an amount of color is metered between the two rolls 35 and 37 which is such that there will be maintained upon the surface of the roll 35, as it approaches the nip and the paper therein, an amount of color suspension slightly in excess of the amount to be applied to remain on the surface of the web 25 as it passes from between the rolls 35-36. Like controlled conditions are effectuated with respect to the color applied to the surface of the roll 36 to be carried up into the nip and to the paper web. The color as introduced to the nip-trough is of very high solids content, ordinarily ranging in commercial operations from approximately 40% up to 56%, generally of the order of 50% or somewhat more, and even somewhat higher than 56% when desired. A color suspension which has been found to function very satisfactorily in the practicing of this invention, utilizing the equipment above described, is of the following composition:

|                 | Per cent |
|-----------------|----------|
| 43 Stayco       | 14       |
| Domestic clay   | 41½      |
| English clay    | 41       |
| Ammonium oleate | 2½       |
| Calgon          | 1        |
|                 | <hr/>    |
|                 | 100      |

Such color gives satisfactory results in the practicing of this invention when admixed with water to having a solids content of approximately 52% to 56%.

A suitable casein containing color, which has likewise been used satisfactorily, is as follows:

|                  | Per cent |
|------------------|----------|
| 60 Casein        | 3        |
| Stayco           | 18       |
| H. T. clay       | 39       |
| Satin H. T. clay | 38½      |
| Ammonium oleate  | 1½       |

"H. T. clay" is an American clay which has long been known in the paper industry, under that designation, and indicates such a clay which has been refined and treated to remove larger particles and extraneous matter, and to improve its color for use in the paper industry as a mineral surfacing material. "Satin H. T. clay" has also been sold by processors of clays for the paper industry and used in the paper industry under that title and is an American clay which

has been processed and treated also to remove large particles and extraneous matter and to give a different grade of clay for use in the paper coating industry, and is prepared generally according to the process disclosed in U. S. Patent to Maloney No. 2,158,987. The term "domestic clay" is used to differentiate clays coming from American clay deposits suitably processed for use in the paper industry, such as the H. T. clay and Satin H. T. clay above referred to, and clays of somewhat different characteristics which have also been long used in the paper industry, including that part of the industry relating to the coating of paper, and which are derived from clay deposits in England.

"Stayco" is a trade-name for a thin boiling oxidized starch made by the Staley Manufacturing Company, a satisfactory oxidized starch as referred to hereinafter.

"Calgon" is a commonly accepted trade name for a sodium phosphate (such as hereinafter referred to) developed for water conditioning, its properties being—specific gravity 2.5; refractive index 1.485. It is insoluble in organic solvents, mutually soluble with water in all proportions. In water solution it binds various metallic ions tightly in soluble complexes, particularly calcium. It coagulates albumens. It disperses finely divided metal oxides and salts. It inhibits crystallization of slightly soluble compounds such as calcium carbonate, and calcium sulphate. And though essentially neutral in solution it reverts to acid orthophosphate very slowly at ordinary temperature and very rapidly about 100° C.

"Ammonium oleate" is a chemical compound, and data with respect to it may be found in any comprehensive chemical text book or dictionary.

The term "consistency" herein is used to indicate that property which may be caused to be present in a liquid suspension or gel by proper selection of its constituents whereby a shearing stress acting thereon produces within the liquid or suspension a change in its state of fluidity or flowability the amount of change having relation to the rate of shear. Viscosity, as the term is ordinarily used to indicate the degree of flowability of a liquid or liquid suspension, should not be confused, herein, with the term consistency; for while the "consistency" and "viscosity" of a given liquid under given conditions may be the same, "viscosity" as used herein is a straight line function, expressed in poises, which does not vary with the rate of shear. Whereas consistency is a variable one, also expressed in poises, in which the variation in poises expresses the ratio of the shearing stress acting on the liquid or suspension to the rate of shear. Or, consistency is that property of a liquid or liquid suspension by which it resists permanent change of shape; and, therefore, if a shearing stress is imposed whereby this resistance is overcome the resultant increase in flowability is the resultant of the ratio of the shearing stress to the rate of shear, as expressed in poises. In other words some liquids, such as water, are of such character that the rate of flowability is substantially constant if other conditions remain the same regardless of what shearing stress may be placed on the component molecules by agitation or stirring and in such the term viscosity, to indicate the flowability, is sufficient, since this is a non-variable characteristic. But in liquids or liquid suspen-

5  
1015  
2025  
30  
3540  
45  
50  
5560  
6570  
75

sions such as the mineral suspension used herein the constituents and the inherent characteristics thereof may be made such that impressing a shearing stress thereon causes a variation in the fluidity and flowability—and with thixotropic materials the flowability is a variable curve function with the increase in flowability being determined as the ratio of the shearing stress to the rate of shear which it produces, and the magnitude of the ratio (and the increase in flowability which is the result) is measured by the rate of shear which is produced in the liquid. We have found that in certain liquid-mineral suspensions, a very thick suspension which ordinarily would be termed very viscous or non-flowing mineral colors, in the paper making industry, may be changed by such shear working, as by a rotating roll and the shearing stress it produces, to a fluent readily flowing one.

The consistency of the color at this point in the invention should be such that despite its high solids content it may be pumped through the nozzles 119—119' and to spread out to give uniform distribution and head throughout the pool in the nip-trough. Furthermore, its trixotropic characteristics are controlled by the uniformly admixed constituent materials so that the working in shear from the contacting rolls will change its state of flowability as metered to one having a viscosity reading of as low as 50 poises or less—the first example given above having its viscosity reduced at the metering nip to approximately 32-33 poises in actual commercial operations despite its high solids content and normally high viscosity. This action is immediately to reduce the viscosity of the metered color and to complete the coating action so that the color metered onto the application rolls will be applied to the paper web, and will flow or spread readily and uniformly on the paper web under the action of the application rolls and will even flow to some extent on leaving the nip and separating from the roll to give uniform and smooth film surface, despite its high solids content and comparatively low water content before it reverts to its normally high viscosity. This is accomplished by preparing the color suspension of materials so selected and processed that the unusually high flowability with respect to high solids content is attained by predetermined working in shear and is coordinated with the characteristics of the web, its speed of travel, the character of the rolls and the relative adhesion tension.

In each of the color suspension formulas set out above a material, such as the sodium metaphosphate specified, is used which has a deflocculating effect—i. e. a comparatively small amount thereof very substantially increases the flowability or fluent characteristics and the wetability, so to speak, which means the capacity of the fluid to wet the paper web despite the restraining forces which would otherwise be effective in a suspension of such high solids content.

In addition the color composition is chosen to be of high thixotropic character so that the material may be quickly brought from its normal condition of high viscosity and impractically low flowability to a condition of tremendously increased fluidity and flowability predetermined as satisfactory for the various controlling operating conditions. Thixotropy is determined

as to its degree by means of a scientific instrument known as the McMichael viscosimeter, a known scientific instrument. Through the use of this, consistencies are determined at two different speeds of the instrument and may then be calculated to give the degree of thixotropy. In the present invention thixotropy is expressed as the ratio of consistencies (i. e. relative viscosities) at 4.5 R. P. M. to 40 R. P. M.; and in the illustrations of color consistencies given above the first formula gives a consistency at 4.5 R. P. M. of 80-135 poises and at 40 R. P. M. of 20-50 poises. This gives a thixotropy, expressed as the ratio of consistencies of 4-2.7. The second formula gives a consistency at 4.5 R. P. M. of 75-120 poises and at 40 R. P. M. of 16.5-26 poises for a thixotropy of 4.55-4.53 which is to say that the constituents of the color suspension have been so chosen and compounded that when subjected to the successive processing steps and maintained in uniformity of condition at the nip-trough the final working in shear at the metering nip will deliver the metered quantity of color to the paper at the nip of the application rolls in said state of relatively high fluidity and flowability, despite its very high solids content, and will permit of securing the required uniformity of distribution upon and incorporation with the surface zone of the paper web. The above reference to the use of the well known McMichael viscosimeter acting at two arbitrarily selected speeds of 4.5 R. P. M. and 40 R. P. M., upon the two color formulations set forth above, and more specifically described later in the specification in connection with the description of the manufacture of the coating color starting with the constituent materials, is merely for illustrative purposes; and the different viscosity readings for each coating color at the two arbitrarily chosen speeds of 4.5 R. P. M. and 40 R. P. M. represent the viscosity readings of a McMichael viscosimeter at the two operating speeds indicated acting upon each particular color formulation. And from those two readings the ratio of consistencies can be determined as stated, and these ratios will indicate decreases or increases in viscosity readings which would be shown for either higher or lower R. P. M. of the McMichael instrument. It is, of course, well understood by skilled physicists and physical chemists and others scientifically and technically skilled in the practical manufacturing fields of industry that the viscosity reading indicated by the McMichael viscosimeter for liquids or suspensions which have varying viscosities at different rates of shear is according to a scale, and if the R. P. M. of the McMichael were reduced below 4.5 then the viscosity reading for the two color formulations would increase according to the thixotropic characteristics of those color suspensions and, likewise, if the R. P. M. were increased above 40 the viscosity reading for each of the color formulations referred to would decrease below the illustrative figures given for 40 R. P. M. It is evident, however, from the explanation of "consistency" as used in connection with variable or temporary viscosities in a thixotropic suspension, due to working in shear, that the rate of change in viscosity as the speed of the measuring instrument is increased or decreased will vary according to the constituents. Thus it is evident that the ratio of consistencies stated as determined in the coating color suspension of

the first formulation referred to will vary over a wider range than is the case with the second formulation which uses casein as an adhesive. This discussion shows clearly to one skilled in the field of coating paper webs, that a color suspension of substantially the same solids content but having a phosphate such as Calgon which falls within the group of alkali phosphates, as referred to in column 16, and which materials are recognized herein as dispersing agents for controlled affect upon the thixotropic characteristics of the coating color suspension, has such effect upon the suspension of minerals and starch adhesive that varying the rate of working in shear will cause greater variations in the viscosities corresponding to varying rates of working in shear than is true with a coating color suspension using casein as an adhesive, although the casein itself is recognized as having such substantial dispersing powers so that the phosphates need not necessarily be used. And by adequate working in shear under high pressure for even the short time interval during which the coating color is subjected to working in shear at the metering nip and also at the color applying nip, actual temporary viscosities are attained, with such high solids content compositions, that the temporary viscosity will be brought down to a reading as low as 1.1 to 1.7, as fully disclosed, mathematically and by discussion of principle of operation, in the copending application of Rudolph N. Griesheimer, Serial No. 436,371, filed March 26, 1942, now Patent No. 2,392,662 issued January 8, 1946. The viscosity readings given for illustrative purposes in explaining the ratio of consistencies, above, are not intended to be limiting in any way except as indicating a range of viscosity readings well within the capacity of the long available McMichael viscosimeter, to permit the manufacturer of coated paper webs to determine that sufficient drop in temporary viscosity could be secured through working in shear using the principles of the present invention and the preferred embodiment of mechanism disclosed, despite such high solids content as would have been considered entirely impossible and impractical to be used with any form of coating mechanism, or any process of coating, prior to applicants' invention.

In connection with each of the nip-troughs a dam or weir 160 is provided at each end of the nip-trough so that the level of the mineral suspension, and therefore the head at the metering nip, can be maintained as desired. In actual practice satisfactory results have been attained with a head of about 22½ inches in the nip-trough. Any excess is led away, and if desired can be returned to the machine storage chest. However, with the upper roll 35 the rate of feed to the nip-trough can be so regulated as to substantially correspond to the rate at which the mineral suspension is applied to the paper, but an overflow pipe can be provided if desired or a save-all pan as illustrated in connection with the lower roll 36. In controlling the amount of mineral suspension, in the particular arrangement of rolls shown in Fig. 2, the roll 140 is positioned with respect to the metering roll 37' so as to permit an amount of mineral suspension to go through which is in excess of that which is to be metered onto the surface of the roll 36. As a result the adhesion tension carries this excess upwardly into the lower nip between the rolls 36 and 37', to maintain a substantial excess

or pool therein. It is unnecessary that the amount of suspension being fed into this pool be measured with any extreme accuracy as any surplus merely drips downward and is caught in the save-all pan 161, that pan being supported from the standard 55, and any color dripping into it being returned to the machine storage chest. Under the conditions described and for a paper speed of 450 feet per minute, with a web, or raw stock, of 40 pounds per ream of 500 sheets 25 x 38 inches, having its absorptivity so adjusted with respect to the freeness of the color that at such speed there will be suitable penetration and setting of the color before contact with succeeding rolls, when color solids content and consistency are adjusted with respect to the roll settings, etc., to produce a coat weight of 15 pounds per ream divided equally on the two sides, the headers 115-115' are each satisfactorily of 3" diameter and the pipes 116-118 and nozzles 119 of  $\frac{3}{4}$ -1", and the suspension pumped to the headers to be under a pressure of 2-3 pounds per square inch. By the term "freeness" as used herein with respect to the color suspension is defined the ease with which the color parts with its fluid when in contact with the paper and it is measured or expressed as the time in seconds required for the water to penetrate through a piece of standard blotter paper or raw stock when placed on the surface of the color suspension. A "free" color gives a very low reading while a "slow" color requires a comparatively considerable time for penetration. Generally speaking it may be said that all the constituents of the color may have effect upon the freeness and by suitable selection and preparation the freeness may be varied within desired practical limits. Ordinarily the minerals and adhesives used have the most pronounced and easily controllable effects upon freeness. The actual effect in many instances must be determined by actual trial. For example freeness attendant upon any clay may depend entirely on the source and method of manufacture of the clay. Bentonite, which is a very hydrous clay of itself has high water-binding power and therefore tends to give low degree of freeness, whereas a calcined secondary kaolin such as that known commercially as Satin-tone has very little, or practically no, water binding power and so tends to high freeness. Other clays generally fall between these extremes. Also the method of dispersing the clay can change its freeness and the transfer of adsorbed water from clay to starch, and vice versa, may completely reverse the water-binding power, or freeness, of the system. Thus a clay which is very free when dispersed in water may result in a very slow coating color upon addition of starch, and, conversely, a slow clay may result in a free color upon addition of starch. The freeness of the finished color can not be predicted from the freeness of the various components but is the result of the combined actions of the various constituents in the presence of and upon each other. Generally speaking, crystalline minerals, such as calcium carbonate, gypsum, blanc fixe, etc., which are sometimes used in coating suspensions increase the freeness of the color, and are all comparatively very low in water-binding power.

Likewise, the water-binding power of adhesives depends upon several factors. Starches are hydrophylic (have high water-binding power) in character and bind water quite readily. But the extent of the water-binding is dependent on the kind and amount of conversion given the starch

5

10

15

20

25

30

35

40

45

50

55

60

65

70

in preparing it for use. In general, the greater the extent of conversion, the higher the freeness. Addition of other materials such as clays or certain chemicals (such as borax or formaldehyde) will change the freeness of starch appreciably. Casein is another hydrophylic colloid used as an adhesive in coating colors. The freeness of casein is dependent on the method of solution. (This is also true of other properties of casein, such as viscosity, oil adsorption, adhesive strength, etc.) The addition of other materials to casein solution, as with starch, results in various changes in freeness.

In practice, the freeness of coating colors may be adjusted between fairly wide limits by proper choice of materials. If a slower color is desired, bentonite or under-converted starch may be added to bring about this result. To produce a free color, such things as carbonate or other crystalline minerals may be used, or a clay with an inherently lower water-binding power may be selected.

In any event, the best operation is obtained in the practicing of this invention when the freeness of the coating color is adjusted to the absorptivity and receptivity of the paper stock being used as described herein. If other conditions are the same and the same end product is desired a very receptive paper web requires a slow color, a resistant sheet requires a free one. The range of freeness used satisfactorily in actual operations has been from 20 to 80 seconds, and very satisfactory operations being secured in commercial operations with a freeness of 35-40 seconds at the first mineral application device and 30-35 seconds at the second, measured as above described.

The upper roll 35 is driven with a motor 155 which has control means which causes it to drive the roll to give a surface speed which approximately corresponds with the surface speed of the paper passing through the nip. This motor drives this roll through an impeller shaft 156 having universal joints therein and a reduction gear, to permit of adjusting movement of the upper color application roll with respect to the lower while permitting adequately controlled driving thereof. The lower roll 36 is also driven at substantially this same speed by means of the motor 158 and connecting drive shaft 159 and reduction gear; but where rolls of such substantially varying hardness in their surface layers are used, as described above, and under the pressures referred to herein, the deformation of the softer surface layer may result in such variation of roll diameter that appreciable variations in rotational speed may be required to give surface speeds sufficiently alike to get the desired operating conditions although material variations in surface speed in the nip may occur without any objectionable operating results provided the speed variation of a roll surface and the paper surface cooperating with it do not differ by too wide a margin. In the actual commercial operations herein described the rolls 35 and 36, under pressures giving a nip width of approximately  $1\frac{1}{2}$  inches, as described, are driven at such speed that the upper roll has a normal surface speed of approximately 5 feet in excess of the surface speed of the lower roll.

The lower roll 36, in the particular machine described and operated, is driven by the individual motor 158 which is interconnected by suitable synchronizing control, with the synchronizing mechanism for the remainder of the paper ma-

chine, so that this particular roll will have a surface speed properly coordinated with the speed of travel of the paper web 25, as it travels through the machine. Any usual form of accurate synchronizing mechanism may be used for this purpose and therefore it is shown only diagrammatically and designated by the numeral 180.

When it is the lower roll 38 which is connected with the synchronizing mechanism in this manner, the upper roll 35 will then be driven by the individual motor illustrated diagrammatically and marked 155, any suitable form of motor control adequate for giving the desired rotational speed to the upper roll with respect to the paper speed and the speed of the lower roll being usable; and on the roll 35, as with each of the other rolls which is movable in operation or adjustment, some suitable form of universal connection in the drive, such as that described above, should be utilized. The motor drive for this upper roll is preferably so controlled that the surface speed of each of the color application rolls 35-36 is substantially the same as the paper speed. The rolls 37, 37' and 140 each is likewise driven by an individual motor designated respectively by the numerals 162, 163, 164, having suitable speed and torque control so that definite surface speed relations may be maintained as desired between any two cooperating rolls, to maintain such speed and energy transfer relationships at the nip as to provide predetermined working in shear to the color and prevent objectionable variation in the consistency of the color suspension as a result of such additional shear working at the nip.

It is, generally, desirable that the paper enter the nip of the color application rolls by going straight in with substantially the same surface contact on each side as it enters. However, this condition is extremely difficult of attainment, and for practical operations very satisfactory results have been attained with the arrangement shown in Fig. 2 wherein the roll 112 is positioned only a short distance in advance of the nip and the paper web passed thereover so that it is brought into the nip at a slight angle and preferably contacting the harder of the two rolls. Furthermore, because of irregularities in the sheet due to irregular stretching or expansion as the formed paper web is being dried while passing through the machine which ordinarily causes the central part of the paper web to lengthen with respect to the edges, it is desirable to have the roll 112 provided with a substantial crown which facilitates feeding the paper smoothly and without any wrinkles into the nip.

In addition it is desirable that the paper go directly out from the nip on the exit side as wrapping of either roll tends to introduce irregular and unpredictable conditions of worming, pitting, lining and the like, each of which conditions is indicative of lack of desired smooth finish in the mineral surface. As shown each member 48 has a depending support 170, carrying suitable bearings for rotatably supporting a roll 171, this roll being positioned a suitable distance from the nip of the color application rolls, and located so as to lead the paper directly away. Also this roll is preferably water cooled. As thus located the water cooled roll tends to cool the air and collect a film of condensed moisture on its surface which acts to prevent the mineral material upon the surface of the paper from adhering to it and gives that mineral surface an adequate time properly to set, due to the absorptive action of the paper, the thixotropic character of the color, 75

its freeness, etc., before the mineral treated surface passes into contact with the first drier roll 21.

Whereas in feeding the paper into the nip it is preferable to feed the paper as shown in Fig. 2 to slightly wrap the upper, hard roll in order to avoid fluttering or dancing of the paper which is apt to occur if the web is merely led directly into the nip, in leaving the nip it is found that the paper has a definite tendency to wrap one roll in preference to the other, usually the hard or wetter roll, and furthermore that wrapping of a roll gives increased tendency toward the irregularities mentioned. This tendency, as a result of the adhesion tension is sufficient to cause the paper to wrap one of the rolls, at least at times, despite the utilization of the roll 171, which is positioned sufficiently far from the nip of the rolls to avoid defacing the mineralized surface after it is properly applied. To overcome this tendency, perforated or slotted air pipes 180 are located closely adjacent the exit of the nip to blow air against the opposite sides of the web and thus cause it to lead out of the nip without dancing or wrapping. The pipes are spaced slightly apart to permit free passage of the paper web between them without contacting either. Each of these air pipes 180 is connected to a suitable source of supply of pressure air so that a flow of air is introduced into the nip on each side of the paper web and between the web and each roll to provide sufficient air buoyancy to float the web directly out from the nip and prevent any objectionable tendency to follow either roll. While this arrangement is not necessary, the conditions at the exit of the nip should be so controlled that objectionable wrapping of either roll, with undue worming and the like, beyond the inherent capacity of the color to flow to subsequent smoothness, should be avoided. As shown each member 180 is a pipe extending across the machine with either a slit therein or holes so that a sheet, or a plurality of streams, of air may be introduced. Furthermore, when desirable and especially for higher speeds, means are provided, one on each side, so as to blow drying hot air upon the mineral treated sheet to cause more rapid drying and setting of the web before it passes to the first drier roll. The surface of the sheet as it leaves the nip of the color suspension application unit is wet and tacky and sufficient time or treatment must be provided in order that this condition may be so modified that there will not be objectionable depositing of the color on the drier rolls. The air drying and setting of the color to secure this desired operating condition is due in part, of course, to mere evaporation of the liquid as the paper passes through the atmosphere; but at the high paper speeds used this is greatly expedited by the air flowed against the surface and the character of the color as to its evaporation. Also the receptivity of the sheet and the freeness of the color must be so adjusted relatively that there will be sufficient, prompt, penetration of the water and adhesive into the paper web to produce a good bond between coating material and raw-stock, the absence of which results in scaling and flaking of the mineral surface. By properly controlling the freeness and paper web characteristics the color and the air drying satisfactory drying and setting may be secured to avoid any objectionable effect of the drying rolls on the mineral surface.

The mineral suspension or color hereinabove

referred to, which is delivered into the nip-trough between the rolls 35 and 37 and between the two rolls 37' and 140 is carefully prepared to have the composition and characteristics as to consistency, flowability, freeness, etc. as above described in coordinated relationship with respect to the web of paper which is being treated. Apparatus for preparing this suspension is illustrated diagrammatically in Fig. 6. As stated above the suspension has its various constituents selected, each with respect to the other, to give the conditions in operation which are desired to produce the proper end product.

A suitable paper making clay, of proper selected grade, is preferably used, especially where a mineral suspension is desired which has less freeness than would be true with a suspension utilizing finely divided calcium carbonate to control its freeness, such as a carbonate precipitated under controlled conditions to give the finely divided material which is to some extent used in the paper industry. Also English clays, generally speaking, are preferable to domestic clays where the formation, compacting and smoothing, of the paper sheet are less satisfactorily performed with respect to smoothness of surface inasmuch as these clays seem to be somewhat more readily deformable in their response to calendering and therefore these clays seem more readily to spread under calendering action to tend to fill up some of the uncorrected irregularities resulting from undue irregularity in the surface of the sheet, even after the mineral suspension has been dried to specified commercial moisture percentage of 3 to 5%. However, it is especially desirable that the paper web be so formed that its irregularities, as to depth and also as to lateral extent and quantitative capacity of any depressions, shall be maintained within dimensions or limitations which are within the quantitative dimensions as to thickness of applied layer of mineral suspension and the volume thereof available for lateral spread. It is not at all essential that the mineral suspension metered on to the color application rolls 35 and 36 be spread as a uniform film thereacross, but on the contrary the suspension may be in quite apparent ridges, of irregular spacing, provided the mineral suspension is of such character and the surface irregularities of the paper web of such limited depth and lateral extent that the quantity of mineral thus metered upon the surface of the applying roll may be suitably and uniformly spread as the paper passes through the nip to give the desired uniform film.

For purposes of illustration the preparation of the mineral suspension will be described with relation to the utilization of a domestic classified clay such as that known commercially as Satin H. T. and a No. 1 grade English coating clay as mentioned in the illustrative formula above both being selected for their flow properties in the suspension. Referring to Fig. 6 a suitable clay mixer 200 is provided, which has kneading devices therein for thoroughly mixing and kneading the ingredients introduced into this mixer. With reference to actual operations successfully used commercially under this invention and which give color formulas approximately those illustrative ones set out in column 14, the clay is fed in desired amount into the kneading machine 200. For a 2000 pound batch of suspension of the formula referred to above approximately 1700 pounds of clay dry weight is introduced into the mixer 200 along with approximately 60 gallons of water. At the same time a mixture of a suitable dispersing

75

agent, such as the compound of the chemical group known as alkali phosphates, such as sodium meta phosphate or sodium pyrophosphate, a satisfactory commercial dispersing agent of this group being that known commercially as "Calgon," is mixed up in the agitating vessel 201, at a concentration of approximately 2 pounds of Calgon per gallon, which makes sufficient dispersing solution for several batches of mineral suspension having the clay content mentioned. 10 gallons of such Calgon mixture (the equivalent of 20 pounds dry weight) is added to the clays and water in the mixer 200, where the several constituents are mixed for approximately a half hour.

Meanwhile a solution of starch, which may be one of the relatively thin boiling starch such as that known commercially as "Stayco," which is an oxidized starch, has been prepared by introducing 3000 pounds of starch into the starch wetting tank 210, where the 3000 pounds of starch is agitated in 510 gallons of cold water for 30 to 60 minutes. The starch is then pumped, by means of a pump such as the centrifugal pump 211 into the starch cooking tank 212 where live steam is added through the pipe 213 and the mixture of starch and water is cooked up to a temperature of 95° C., this maximum temperature being maintained for approximately 15 minutes. The starch is agitated and thoroughly mixed while cooking, and is preferably passed through a suitable screen such as a rotary screen, before it is fed into the cooking tank. The quantities just mentioned makes sufficient starch for about nine batches of mineral suspension for the paper speeds, coat weight, etc. described above. Having been thus cooked, 108 gallons of this cooked starch (300 pounds dry weight) are dropped by gravity into the starch cooling and measuring tank 215, which is provided with an agitator, 215', capable of keeping the starch thoroughly agitated. From this tank 215 a part is fed to the mixing tank 200 by means of a suitable pump 216 through the pipe 217. Satisfactory results are secured by adding 35% of the batch of starch at this stage which equals approximately 37½ gallons or approximately 105 pounds dry weight. The starch when thus introduced facilitates emptying the clay which has been thoroughly kneaded in the comparatively small percentage of water, the mixture being dumped from the tank 200 into the clay make-down tank 220 which also has agitating or mixing mechanism 220'.

Meanwhile a suitable mixture having lubricating properties has been prepared in the tank 221, oleic acid being a suitable such lubricant. Ammonium oleate is likewise suitable. In preparing this lubricating agent, ammonium oleate for example, it is mixed in the proportion of 2 pounds per gallon, with suitable agitation by the agitating mechanism 222 of suitable high speed agitating type, a similar form of agitating mechanism 201' being used in the tank 201. Of this mixture 25 gallons is now added to the clay mixture in the tank 220 and resulting mixture agitated for approximately 15 minutes. This material effects desired controlled modification of the adhesion-tension of the suspension for the roll surfaces, and causes proper decrease in the tendency toward wrapping the roll and likewise greatly decreases the tendency toward worming which has been found to accompany too great adhesion-tension. This mix is then dropped into the blend tank 225, through a suitable wire basket screen, and in this blend tank the balance of the starch withdrawn as a batch into the tank 215 is added

and the mixing continued, with thorough agitation by the agitator 225', and in this tank for a period of 2 hours. This agitation, with the materials used, gives a working in shear which greatly decreases the consistency and so increases the flowability of the mineral suspension, as a concomitant of its predetermined thixotropic character, and after this mixing in the tank 225 the material is pumped by means of a positive displacement pump of the type known commercially as "Moyno" and as indicated diagrammatically by the numeral 226, the material being pumped through the pipe 227 to a roll mill 228.

This mill 228 may be of suitable character, such as those used in various industries for working pigments in suspension, such as the well known so-called "ink mill." The blended color from the pipe 227 flows into a hopper 229 and then through the rolls of the mill where the milling tends to reduce any objectionable oversize or aggregate particles, remove entrapped or occluded air and still further to blend the starch, pigment and other constituents into a more homogeneous mix, and also to add additional working in shear to prevent reversion and maintain the suspension at the desired condition of consistency for this stage. The milled color flows by gravity through an intermediate tank 235, having a sloping bottom, no agitator being necessary to use in this tank. This sloped bottom feeds the material by gravity toward the discharge outlet to which is connected the inlet of the pump 236, also suitably the so-called "Moyno" type, which pumps the material to the machine storage tank 248 which is substantially a duplicate of the blend tank 225 and has a suitable agitating mechanism 248' as indicated in dotted lines, for maintaining the suspension in thoroughly agitated condition. From the tank 248 the material is pumped by another Moyno pump 245, through the pipe 251 which in turn is connected to the inlet end of the manifold 115 and thence flows through the associated mechanisms at the desired rate controlled by the setting of the valves 117 into the nip-trough. A coating color as so prepared has a solids content within the range of 52-56%, and approximately 53%. Preferably suitable strainers are located in the pipe 251, two of these strainers being shown, the strainer 268 being of the so-called "Sarco" type, which is a commercially well-known apparatus, this strainer being driven by the motor 261. This Sarco strainer has two outlets one connected to the pipe 115 and from that to the manifold 115' this outlet serving to pass the desirably selected material, the other being connected to a pipe 262 through which any rejects may be passed into the save-all pan 161. Likewise a by-pass pipe 251' is provided having a hand operated Sarco strainer 268' which has two branches connected respectively to the manifold 115 and to the reject pipe 262, so that the hand strainer may be used alternately or at the same time with the motor driven one. Preferably the motor driven strainer 268 is used, but after a reasonable period of use, usually about eight hours where the other operations in the preparing of the suspension are adequately carried out, the strainer is cleaned and at such time the hand operated strainer in the by-pass pipe 251' may be utilized while the motor driven strainer is being thus cleaned.

If it is desired to use casein, as in one of the illustrative formulas set out above, the procedure is similar to that described above. Under such

conditions the casein is prepared in the casein kettle 270. Cold water is first added to the casein kettle through the pipe 271 in the proper amount for cutting the casein according to the color formula chosen and the casein is then introduced. The water casein mixture is mixed for 30 minutes, after which the alkali is added and steam turned on through pipe 272. Cooking is continued until the temperature reaches 40-45° C. The casein is then cooled gradually and can be dropped from the casein kettle into the blending tank 225, in the desired proportion.

A pipe connection 273, with pump 274, is provided leading from the casein kettle 270 to deliver into the kneading mill 280, through which a small, controlled portion of the casein may be used with the clay and water in this mixer 280 to act as a dispersing agent—satisfactory results being attained through the use of 3% of the total constituents employed.

Preferably measuring tanks 280, of proper volume, are used to facilitate feeding the liquid ingredients.

The excess color from the nip-trough, and from the save-all 161, is returned to the machine storage chest 248, as indicated at 275. By means of the mechanisms thus described the composition and characteristics of the mineral suspension is maintained uniform, and under uniform head, entirely across the nip-trough and the excess color is returned to the machine chest where the agitation thoroughly mixes it with the other mineral within this chest so that the suspension maintained in the nip-troughs and metered to the color application rolls 35-36 is always of the predetermined character adapted to the characteristics of the paper web, its formation, its receptivity and absorptivity, and the nip pressure.

The pressure between each metering roll 37 and 37' and its corresponding color application roll 35-36, should be accurately adjusted to give the operating conditions desired the mechanisms described above giving extraordinary nicety of adjustment of the order of 4 pounds per linear inch. The quantity of solids applied to and upon the paper web as it passes through the nip is best controlled by properly controlling the solids content of the suspension. However, the pressures at the nip of the rolls 35-36 must be maintained within suitable operating range for most desirable results, the best results for wide variety of conditions being of the order of 90-175 pounds per linear inch. The pressures at the nip are critical in that there is a certain minimum pressure for a sheet of given characteristics below which satisfactory operations will not be secured, but a rough surface will ensue with insufficient spreading and equalizing of the coating as applied to the paper. This minimum has been found to be about 40-45 pounds per linear inch for papers made from a furnish such as described above, and with rolls having the surface layers of the character described but for satisfactory commercial operations pressures substantially in excess of this minimum, and generally within the range of 90-175 pounds specified, are preferably used. Also there is a critical upper limit of pressure above which increases produce a pattern of the raw stock irregularities and also may effect the inherent characteristics of the sheet under the pressures and with the conditions of the sheet under its absorption of fluids and the like, so that undesirable blackening may show up in subsequent calendering. Such poorer results

have been obtained in operations using pressures above 275 pounds per linear inch.

A color suspension of the first formula specified above will have a solids content of approximately 56%, and with this suspension the paper may readily be coated to provide a coat weight of 15 pounds per ream of 500 sheets 25x38 inches divided equally upon the two sides of the paper. By increasing this percentage of solids even heavier coats may be applied satisfactorily.

If it is desired to apply a second coat, which may be particularly desirable where very heavy weight coats of the order of 20 pounds or more divided equally between the two sides are to be produced, an additional color applying mechanism may be utilized as illustrated in Fig. 1A, where the color application rolls are indicated by the numerals 35" and 36", the other parts of the mechanism being the same in construction as those heretofore described. Where this second coating operation is to be used the formula of the mineral suspension is somewhat different from that used on the first inasmuch as satisfactory results may ordinarily be more readily obtained if this second coating is of somewhat lighter weight than the first and also if the color has somewhat less mineral and more adhesive or sizing material. For a single coat, as described above, the solids contents will ordinarily be satisfactory if ranging from 52-56% of solids with starch as the adhesive. The formula for the second coat contains also casein and on this account, and for the reasons described above, the second formula contains a smaller quantity of solids, of the order of 43-45%, and the somewhat increased percentage of adhesive. Also quite satisfactory results and end products may be attained if the mineral suspension first applied is of a formula comprising nearly all of the mineral solids applied and a greatly reduced amount of adhesive, and the suspension applied as the second step comprises only a small amount of mineral and nearly all of the adhesive or sizing constituent. For example, the formula for the first treatment may satisfactorily comprise 52-56% of solids; with the second treatment formula containing 43-45% of solids. We have found that such high mineral-low adhesive constituent will give a mineral surface which is quite smooth and has great reduced tendency to worming, etc. Where a second coating treatment is applied the paper is then passed through the additional drying unit illustrated and containing the same sort of drier rolls 27 and is dried to the desired final moisture content, preferably around 3 or 4 to 6%.

After its final coating operation, whether a single coat or double coat, the dried paper is then usually passed through a suitable final machine calender stack indicated generally by the numeral 300 where it is subjected to nip pressures of the order of 195 to 215 pounds per linear inch.

As stated above the metering rolls should be adjusted so as to give very accurate metering of the quantity of suspension passing the metering nip and traveling thence upon the surface of the roll to be carried around and brought into contact with the traveling web of paper at the nip of the application rolls 35-36. If less than the desired amount of mineral is carried to the nip, for any suitable length of time, even though the deficit be very small in quantity, the receptivity of the paper surface being therefore in excess of the quantity of mineral suspension applied to it, an unsatisfactory surface will be

secured since it will be non-uniform and even discontinuous, and also not adequately smooth. If this inadequate supply is continued for any length of time the rolls 35-36 tend to run completely dry on the surfaces and this in turn tends to cause the rolls to be irregularly sticky with respect to the color and to thus make an uneven and irregular application of color upon the paper as it leaves the nip of the rolls. In actual practice the metering rolls are accurately controlled so that somewhat in excess of the amount required to be applied to the paper will be on the surfaces of these rolls beyond the metering nip to be carried on into the nip against the paper. By properly coordinating the composition and characteristics of the mineral suspension, the receptivity and absorptivity of the paper, and the uniformity of spreading and distribution of the color in and upon the paper as it passes through the nip, a very limited, lubricating quantity of the suspension will remain upon the surface of each roll as it leaves the nip; which quantity, when the various controlling conditions are properly coordinated, apparently becomes a substantially constant factor and provides that very slight excess which is carried into the nip and which, though very slight, is sufficient to prevent the rolls from running dry, or from becoming irregularly dry with the attendant difficulties described. When such operations are satisfactorily in progress the surfaces of the rolls 35 and 36 are wet or moist with this slight excess of color after the paper with its applied layer of color at the exit of the nip has moved away and out of contact therewith, a desirable and satisfactory operating condition being indicated where these rolls as they leave the nip are thus lubricated or moist on the surface.

Also, as stated, it is not necessary that effort be made to utilize the metering rolls 37-37' for applying a continuous and uniformly spread film of the metered color suspension across the faces of the rolls 35-36. In fact, it is unnecessary to even approach such a condition, and in satisfactory commercial operations referred to and with the formulas, meter pressures, etc. described the metered color upon the faces of the rolls 35-36 as it moves up to the nip and is brought into contact with the paper entering the nip is readily observed as being ridgy and of non-uniform depth. In fact, satisfactory results have been secured where the metered color being carried to the nip is discontinuous, being in ridges which are either completely or substantially unconnected by a thinner film of color. This may be indicated by lifting the roll and applying a sheet of paper to it as it approaches the nip whereby a discontinuous pattern may be transferred onto the paper. But for satisfactory operating conditions it has been found that the solids content, the consistency and the nip pressures for the suitable raw stock should be so controlled that at the nip where the color is applied to and spread upon the paper the ridges and irregularities and the general distribution shall be such that the color suspension will be flowed to blend and equalize uniformly across the paper web under such pressures. When a color is used of suitably controlled characteristics with respect to the paper to be of high flowability after its application to the paper as it moves from the nip, additional flowing and equalizing occurs, even sufficient with some colors to produce smoothness of finish despite obvious irregularities at the point of exit.

While the methods and forms of apparatus

herein described constitute preferred embodiments of the invention, it is to be understood that the invention is not limited to these precise methods and forms of apparatus, and that changes may be made therein without departing from the scope of the invention which is defined in the appended claims.

What is claimed is:

1. In coating apparatus of the character described the combination of a pair of rolls forming a nip-trough, means for supply a coating color thereto to effect formation in said nip-trough of a uniform and homogeneous coating mass, said means comprising a plurality of spaced discharge nozzles connected to a source of coating color and located to discharge quantities of color directly into the nip-trough, and means for reciprocating said nozzles longitudinally of said nip-trough with a predetermined stroke to provide for introduction of the coating color to said nip-trough to maintain a body of color of predetermined depth and in a substantially uniformly distributed manner.

2. In the manufacture of paper of the character described having a mineral finished surface adapted to receive printing impressions; the method which comprises passing a paper web between the traveling surfaces of color applying rolls, maintaining a substantial pressure of not less than about four pounds per linear inch across the application nip of said rolls; supplying a mineral and adhesive coating color comprising essentially coating pigment and an adhesive and a lubricating agent therefor and having solids content of not less than about 40-56%, and which coating color is of high thixotropy and is normally highly viscous or non-flowable and at 40 R. P. M. of a McMichael viscosimeter has a viscosity reading of approximately not more than 50 poises in a maintained quantity to be conditioned, subjecting said maintained color to high shear working to cause large decrease in viscosity of said color to temporarily low viscosity and fluid condition, metering said color while maintaining said temporary low viscosity condition across the surface of one of said applying rolls, the amount of said color metered to said color applying roll being controlled to all pass through the application nip with the traveling paper web and in limited excess of that to remain as a coating on the web, the pressure at the application nip being maintained substantial and such as to cause pressure distribution and blending of the metered color on the web, and causing adhesion separation of said excess color from the amount of color carried away from the application nip on the paper web, said separated excess adhered to the application roll and being carried by it away from the nip and admixed with the conditioned color prior to completion of the metering.

3. The method in the coating of a web of paper to produce a printing surface, through the utilization of coating means, comprising conditioning and metering rolls and application rolls, and a highly thixotropic suspension of coating color comprising mineral pigment and adhesive and of predetermined high solids content of not less than about 40 to 56% solids and which color normally is in highly viscous or substantially non-flowable condition, such that at 4.5 R. P. M. of a McMichael viscosimeter it has a viscosity reading of not less than about 75-135 poises and at 40 R. P. M. of the McMichael viscosimeter not more than about 16.5-50 poises, which comprises supplying a maintained quantity of said coating

color to the coating conditioning and applying rolls, subjecting the normally highly viscous or substantially non-flowable color to high shear working by the traveling surfaces at the nips of the conditioning and metering rolls and color application rolls to effect temporarily a large drop in viscosity to change the color into fluid and readily flowable condition, maintaining said condition for a limited operating time, metering said conditioned color between the traveling surfaces of said metering and conditioning rolls while urging said rolls toward each other to provide metering surfaces separated from each other by said conditioned color under high pressure effective on said color of not less than 4 pounds per linear inch of roll length, said metering being accomplished in two successive high shear metering operations under said substantial pressure and said second metering operation being effective upon said metered color from the first metering operation while its metered condition is maintained, and applying said conditioned and metered coating color in said metered condition continuously to said traveling web of paper as the paper and metered quantity of color pass through the color application nip between said application rolls and controlled in quantity such that all the metered color will pass into the application nip with the traveling paper web, and subjecting the color to distribution pressure in the application nip to give a uniform blending and distribution of the color applied on the paper while said temporarily fluid condition persists in said coating color, to form a substantially smooth and uniformly distributed coating on said paper.

4. The method in the coating of a web of paper to produce a printing surface, through the utilization of coating means, comprising conditioning and metering rolls and application rolls, and a highly thixotropic suspension of coating color comprising mineral pigment and adhesive and of predetermined high solids content of not less than about 40 to 56% solids and which color normally is in highly viscous or substantially non-flowable condition, such that at 4.5 R. P. M. of a McMichael viscosimeter it has a viscosity reading of not less than about 75-135 poises and at 40 R. P. M. of the McMichael viscosimeter not more than about 16.5-50 poises, which comprises supplying a maintained quantity of said coating color to the coating conditioning and applying rolls, subjecting the normally highly viscous or substantially non-flowable color to high shear working by the traveling surfaces at the nips of the conditioning and metering rolls and color application rolls to effect temporarily a large drop in viscosity to change the color into fluid and readily flowable condition, maintaining said condition for a limited operating time, metering said conditioned color between the traveling surfaces of said metering and conditioning rolls while urging said rolls toward each other to provide metering surfaces separated from each other by said conditioned color under high pressure effective on said color of not less than 4 pounds per linear inch of roll length, and applying said conditioned and metered coating color in said metered condition continuously to said traveling web of paper as the paper and metered quantity of color pass through the color application nip between said application rolls and controlled in quantity such that all the metered color will pass into the application nip with the traveling paper web, and subjecting the color to distribution pressure in the application nip to give a uniform blending and

distribution of the color applied on the paper while said temporarily fluid condition persists in said coating color, to form a substantially smooth and uniformly distributed coating on said paper constituting a major portion of said coating color and retained on the web as it leaves the nip, and causing adhesion onto the roll surface for separation from said uniformly distributed applied coating of a minor proportion of said coating color carried away from the nip as a lubricating film on said roll surface.

5. In the manufacture of coated paper to provide a printing surface, the method which comprises the steps of supplying at the coating zone a maintained quantity of a coating color including as essential ingredients a finely divided coating mineral pigment and an adhesive, a dispersing agent and a lubricating agent therefor, said color having high solids content of not less than about 40-56% and being highly thixotropic and in normal state highly viscous or substantially non-flowable and having at 4.5 R. P. M. of a McMichael viscosimeter a temporary viscosity reading of not less than about 75-135 poises and at 40 R. P. M. of the McMichael viscosimeter a temporary lower viscosity reading of not more than about 50 poises, subjecting said maintained quantity of color to intense high shear working to change said color into a temporarily lowered viscosity and fluid and readily flowable condition, metering said temporarily low viscosity color under high shearing pressure between contacting curved traveling surfaces across which pressure is applied in excess of about 4 pounds per linear inch along the line of contact, and supplying said metered portion of said color in the metered state to the surface of the paper to apply a uniform coating thereon, while maintaining the proportions of constituents of said color and the temporary low viscosity condition of the metered color when being applied to the paper substantially unchanged.

6. In the manufacture of coated paper to provide a printing surface, the method which comprises the steps of applying to the paper a coating color having as essential ingredients a finely divided coating pigment and an adhesive and a dispersing agent and a lubricating agent and water to provide a substantially homogeneous admixture of high solids content constituting approximately not less than 40-56% and said color being highly thixotropic and in normal state highly viscous or substantially non-flowable such that at 4.5 R. P. M. of a McMichael viscosimeter said color will have a temporary viscosity reading of not less than about 75-135 poises and at 40 R. P. M. of the McMichael viscosimeter will have a temporary viscosity reading of not more than about 50 poises, supplying said color into a maintained quantity at the coating zone, subjecting said highly thixotropic color to intense high shear working at the coating zone to cause a great reduction in temporary viscosity to change said color into a temporarily low viscosity and fluid and readily flowable condition, metering said temporarily low viscosity and fluid and readily flowable color under high shearing pressure between contacting curved traveling surfaces across which pressure is applied in excess of about 4 pounds per linear inch along the line of contact, and supplying said metered portion of said color in the metered state to the surface of the paper and subjecting the color on the paper to a distributing pressure to apply a uniform coating thereon, while maintaining the proportions of constituents

of said color and the temporarily low viscosity condition of the metered color when being applied to the paper substantially unchanged.

7. In the manufacture of coated paper to provide a printing surface, the method which comprises the steps of applying to the paper a coating color having as essential ingredients a finely divided coating pigment and an adhesive and a dispersing agent and a lubricating agent and water to provide a substantially homogeneous aqueous-mineral-adhesive coating admixture with a high solids content constituting approximately not less than 40-56% and said color being highly thixotropic and which is in normal state highly viscous or substantially non-flowable but which is constituted for drastic and substantial temporary viscosity reduction under intense high energy input working in high shear immediately prior to application to the paper web, and such that at 4.5 R. P. M. of a McMichael viscosimeter said color will have a temporary viscosity reading of not less than about 75-135 poises and at 40 R.P.M. of the McMichael viscosimeter will have a temporary viscosity reading of not more than about 50 poises, supplying said color into a maintained quantity at the coating zone, subjecting said highly thixotropic color to intense high shear working at the coating zone to cause a great reduction in temporary viscosity to change said color into a temporarily low viscosity and fluid and readily flowable condition, metering said temporarily low viscosity and fluid and readily flowable color in two successive high shear metering steps under high shearing pressure between contacting curved traveling surfaces across which pressure is applied in excess of about 4 pounds per linear inch along the line of contact, and supplying said metered portion of said color in the metered state to the surface of the paper and subjecting said color on the paper to distributing pressure during the application step to effect blending and smoothing of the color to apply a substantially uniform coating thereon, while maintaining the proportions of constituents of said color and the temporarily low viscosity condition of the metered color when being applied to the paper substantially unchanged.

8. The method of coating of a web of paper to provide a printing surface, through the utilization of the traveling surfaces of coating conditioning and metering rolls and application rolls and a highly thixotropic suspension of coating color comprising mineral pigment and adhesive and of predetermined high solids content of not less than about 40% to 56% solids and which color normally is in highly viscous or substantially non-flowable condition, and at 4.5 R. P. M. of a McMichael viscosimeter has a viscosity reading of not less than about 75-135 poises and at 40 R. P. M. of not more than about 16.5-50 poises, which comprises supplying a maintained quantity of said coating color to the coating conditioning and applying rolls, subjecting the normally highly viscous or substantially non-flowable condition color to high shear working by the traveling surfaces at the nips of the conditioning and metering rolls and the color application rolls to effect temporarily a large drop in viscosity to change the color into fluid and readily flowable condition maintained for a limited operating time, metering said conditioned color between the traveling surfaces of said metering and conditioning rolls while urging said metering surfaces toward each other under high pressure of not less than 4 pounds per linear inch of roll length, and applying said

conditioned and metered coating color in said metered condition continuously to said traveling web of paper as the paper and metered quantity of color pass through the color application nip and controlled in quantity such that all the metered color will pass into the application nip with the traveling paper web, to give a uniform blending and distribution of the color on the paper web while said temporarily fluid condition persists in said coating color, to form a substantially smooth and uniformly distributed coating on said paper.

9. The method of coating a web of paper which has been dried to a moisture content of less than approximately 10%, and which has been calendered to have a compacted and smoothed surface in which the irregularities have dimensions within the thickness of the subsequently applied coating and unit area of flowable coating composition subsequently applied thereto, which comprises the steps of passing said web of paper through the application nip between the traveling surfaces of color application rolls, supplying a coating color containing mineral pigment and an adhesive in liquid suspension of predetermined high solids content of not less than approximately 40-56% total solids, said color being normally highly viscous or substantially non-flowable and highly thixotropic and subject to large temporary reduction in viscosity with change into a fluid and readily flowable condition under working at a high shearing rate and having a temporary viscosity reading at 4.5 R. P. M. of a McMichael viscosimeter of not less than about 75-135 poises and at 40 R. P. M. of a McMichael viscosimeter a temporary viscosity reading of not more than about 16.5-50 poises, subjecting said coating color prior to applying the coating to the paper web to predetermined working under high rate of shear at substantial pressure exerted across said nip, said pressure being of the order of not less than 4 pounds per linear inch of roll length, to change it, for a limited operating time, into a temporary condition of greatly reduced viscosity and concomitant fluid and readily flowable condition, including successive workings in shear under maintained substantial pressures and high roll speeds at two conditioning and metering nips under substantial pressures of the order of not less than 4 pounds per linear inch of roll length with resultant working at a high rate of shear and metering of said temporarily fluid color in controlled amount through each metering nip and onto the application roll to pass directly to the application nip in amount limited to pass with the paper web into and through the application nip and to cause a major amount of said applied wet coating to separate at the exit of the application nip, from a lubricating excess in minor amount, and to be carried from the nip on the web, to form a substantially smooth and uniformly distributed coating on said paper.

10. In the manufacture of coated paper to provide a printing surface and using color application and conditioning and metering rolls, the method which comprises the steps of applying to the paper a coating color having as essential ingredients a finely divided coating pigment and an adhesive and dispersing agent and a lubricating agent and water to provide a substantially homogeneous aqueous-mineral-adhesive coating admixture with a high solids content constituting approximately not less than 40-56% and said color being highly thixotropic and which is in normal state highly viscous or

substantially non-flowable but which is constituted for drastic and substantial temporary viscosity reduction under intense high energy input working in high shear, and such that at 4.5 R. P. M. of a McMichael viscosimeter said color will have a temporary viscosity reading or not less than about 75-135 poises and at 40 R. P. M. of the McMichael viscosimeter will have a temporary viscosity reading of not more than about 50 poises, supplying said color into a maintained quantity at the coating zone, subjecting said highly thixotropic color to intense high shear working at the coating zone to cause a great reduction in temporary viscosity to change said color into a temporarily low viscosity and fluid and readily flowable condition, metering said temporarily low viscosity and fluid and readily flowable color under substantial pressure of not less than 4 pounds per linear inch of roll length, and supplying said metered position of said color in the metered state to the surface of the paper, and subjecting said color on the paper to distributing pressure in the application nip to effect blending and smoothing of the color to apply a substantially uniform coating thereon, while maintaining the proportions of constituents of said color and the temporarily low viscosity condition of the metered color when being applied to the paper substantially unchanged, causing adherence separation of a minor excess portion of said metered portion onto the surface of the application roll leaving the application nip, and returning said separated color to the conditioned color before the metering operation is completed and returning a major portion of said color upon the paper web leaving the application nip as a substantially uniform applied coating.

11. Apparatus of the character described for applying a mineral coating color to a paper web to provide a surface for receiving printing, which includes in combination a pair of application rolls one of which is soft with respect to the other to provide a substantially wide application nip under roll deforming pressure, means for supporting said application rolls constructed for separating the two rolls and for moving them toward each other including a pivotal mounting and means effective for urging said rolls toward each other within a substantial operating pressure range of approximately 4-200 pounds per linear inch of roll length, a pair of color conditioning and metering rolls comprising an outer roll spaced from a first application roll and an intermediate roll between said first application roll and said outer roll, means for pivotally supporting the intermediate roll with respect to the application roll and the outside roll with respect to the intermediate roll, means for urging said outside and intermediate rolls together under substantial pressure to constitute a color receiving trough therebetween, means for feeding color into said trough at a controlled rate, means for urging said intermediate roll conjointly with said outside roll toward said application roll with a selected substantial pressure within said pressure range of approximately 4-200 pounds per linear inch, said first pressure means being adjustable within said pressure range to be effective upon said rolls for metering said color onto said application roll at such rate that said color will pass into the substantially wide application nip with the paper web under said pressure maintained at said application nip, and said mounting and operating

means for said rolls including means interconnecting said intermediate and outside rolls effecting conjoint movement thereof when said rolls are moved away from said application roll, gauge means for showing the selected pressure acting to urge said application rolls toward each other whereby said substantially wide application nip is formed, and gauge means for showing the selected pressure acting to urge said pair of conditioning and metering rolls toward each other and said intermediate roll of said pair toward said application roll.

12. Apparatus of the character described for applying a mineral coating color to a paper web to provide a surface for receiving printing, which includes in combination a pair of application rolls forming a substantially wide application nip under roll deforming pressure, means for supporting said application rolls constructed for separating the two rolls and for moving them toward each other including a pivotal mounting and means effective for urging said rolls toward each other within a substantial operating pressure range of approximately 4-200 pounds per linear inch of roll length, a pair of color conditioning and metering rolls comprising an outer roll spaced from a first application roll and an intermediate roll between said first application roll and said outer roll, means for pivotally supporting the intermediate roll with respect to the application roll and the outside roll with respect to the intermediate roll, means for urging said outside and intermediate rolls together under substantial pressure to constitute a color receiving trough therebetween, means for feeding color into said trough at a controlled rate, means for urging said intermediate roll conjointly with said outside roll toward said application roll with a selected substantial pressure within said pressure range of approximately 4-200 pounds per linear inch, said pressure means being adjustable within said pressure range to be effective upon said rolls for metering said color onto said application roll at such rate that said color will pass into the substantially wide application nip with the paper web under said pressure maintained at said application nip, and said mounting and operating means for said rolls including means interconnecting said intermediate and outside rolls effecting conjoint movement thereof when said rolls are moved a way from said application roll, gauge means for showing the selected pressure acting to urge said application rolls toward each other whereby said substantially wide application nip is formed, gauge means for showing the selected pressure acting to urge said pair of conditioning and metering rolls toward each other and said intermediate roll of said pair toward said application roll, and guide means including guide rolls for controlling the angle of contact of the web with either of said application rolls to induce the web to wrap one of said rolls before entering the nip therebetween, said means controlling both the time during which the web is in contact with the color under pressure in the application nip and the time during which the web is in contact with the color on said application rolls prior to the application of pressure for distributing the color on the web.

13. Apparatus of the character described adapted for manufacturing paper products and imparting a mineral finished surface thereto which is constructed for receiving a color suspension which is highly thixotropic and normally highly viscous or substantially non-flowable and

70

75

contains a predetermined high solids content of the order of not less than about 40-56% of solids and which has a viscosity at 40 R. P. M. of a McMichael viscosimeter of about 50 poises, and which comprises color application rolls, the surface of one of said rolls being soft and deformable by another of said rolls, means for passing a paper web prepared to be treated through the application nip between said color application rolls in which surfacing of the traveling web is to be effected, means for directing the path of travel of the paper web as it passes to and from the application nip comprising a roll to control the angle of approach of the web to the application rolls and a second roll mounted beyond the exit of the application nip for guiding the coated web leaving the application nip, said second roll being chilled for condensation of a layer of moisture thereon, means for separating said application rolls to inoperative positioning and for urging said application rolls toward each other into a contacting positioning for operation to give a predetermined uniform pressure effective upon the web of paper and metered color passing through the application nip of said rolls, means for controlling said pressure means to main said nip pressure within negligible variations of approximately 4 pounds per linear inch of roll length, said pressure deforming the relatively soft surface of one of the rolls by the relatively harder surface of another said roll forming between said rolls a substantially wide application nip, color conditioning and metering means including at least one metering roll and a nip-trough for receiving a maintained supply of said suspension, said metering roll positioned with respect to one other roll to form said nip-trough, means for urging said metering roll toward one of said color application rolls to give a substantial metering pressure in excess of 4 pounds per linear inch of roll length acting upon color passing through the metering nip between said rolls to effect high shear working of said color, means for maintaining a substantially uniform head of said color in said nip-trough, said metering roll subjecting said color in said nip-trough to intensive high shear working before said color enters said metering nip, means for directly reading the pressure between said application rolls, independent means for directly reading the pressure at said metering nip, and means for independently controlling the peripheral speeds of each of said rolls.

14. The apparatus of claim 12 characterized by having at the exit side of the application nip, guide means for the traveling web including guide rolls for controlling the angle with which the web with the coating applied thereto separates from each of said application rolls and for controlling the time during which said web with the coating thereon remains in contact with each of said application rolls after release of pressure applied to said web between said rolls, said guide means comprising means for reducing the temperature thereof substantially below room temperature for providing a lubricating film of condensed moisture thereon to prevent marring and disruption of the smoothed and uniformly distributed surface applied to the web by said application rolls.

JAMES J. O'CONNOR.  
RUSSELL H. SAVAGE.  
HELLMUTH C. SCHWALBE.

## REFERENCES CITED

The following references are of record in the file of this patent:

## UNITED STATES PATENTS

| Number    | Name             | Date          | Number       |
|-----------|------------------|---------------|--------------|
| 730,506   | Adams            | June 9, 1903  | 2,185,859    |
| 744,422   | Smith et al.     | Nov. 17, 1903 | 2,186,874    |
| 1,733,524 | Bradner          | Oct. 29, 1929 | 2,211,348    |
| 1,903,325 | Colbert et al.   | Apr. 4, 1933  | 5 2,236,005  |
| 1,921,368 | Massey           | Aug. 8, 1933  | 2,236,239    |
| 1,933,963 | Bradner          | Nov. 7, 1933  | 2,244,859    |
| 1,951,710 | Schorger         | Mar. 20, 1934 | 2,257,373    |
| 1,964,312 | Bright           | June 26, 1934 | 2,281,340    |
| 2,016,085 | Fawkes et al.    | Oct. 1, 1935  | 10 2,369,378 |
| 2,022,484 | Watkins          | Nov. 26, 1935 | 2,378,113    |
| 2,032,211 | Hornbostel       | Feb. 25, 1936 | 2,425,231    |
| 2,064,776 | Wilkinson et al. | Dec. 15, 1936 |              |
| 2,089,480 | Heritage         | Aug. 10, 1937 |              |
| 2,105,981 | Massey et al.    | Jan. 18, 1938 | 15 Number    |
| 2,151,963 | Flodmark         | Mar. 28, 1939 | 448,578      |
| 2,176,981 | Smith et al.     | Oct. 24, 1939 |              |

| Name             | Date           |
|------------------|----------------|
| Massey           | Jan. 2, 1940   |
| Mason            | Jan. 9, 1940   |
| Nelson           | Aug. 13, 1940  |
| Massey           | Mar. 25, 1941  |
| Lipton           | Mar. 25, 1941  |
| Thiele et al.    | June 10, 1941  |
| Fanselow         | Sept. 30, 1941 |
| Thiele et al.    | Apr. 28, 1942  |
| Thiele et al.    | Feb. 13, 1943  |
| Vander Carr      | June 12, 1945  |
| Dickerman et al. | Aug. 5, 1947   |

## FOREIGN PATENTS

| Country       | Date          |
|---------------|---------------|
| Great Britain | June 11, 1936 |

## OTHER REFERENCES

The Manufacture of Pulp and Paper, McGraw-Hill Book Co., vol. V, 3rd ed., 1939, section 4, pages 2, 21, 23, 24, 27, 28, 31, 36, 38.

**Certificate of Correction**

**Patent No. 2,565,260**

**August 21, 1951**

**JAMES J. O'CONNOR ET AL.**

It is hereby certified that error appears in the printed specification of the above numbered patent requiring correction as follows:

Column 2, line 54, for "apparatus" read *apparatuses*; column 3, line 9, for "solids" read *coating*; column 12, line 52, for "nip-through" read *nip-trough*; column 18, line 57, for "22½" read *2-2½*; column 25, line 63, for "alternately" read *alternatively*; column 33, line 69, before "dispersing" insert *a*; column 34, line 20, for "position" read *portion*; line 35, for "returning" read *retaining*; column 35, line 51, for "a way" read *away*; column 36, line 26, for "main" read *maintain*; column 37, line 21, list of references cited, for "Flodmark" read *Fladmark*; column 38, line 10, list of references cited, for "Feb. 13, 1943" read *Feb. 13, 1945*; line 11, for "Vander Carr" read *Van de Carr*;

and that the said Letters Patent should be read as corrected above, so that the same may conform to the record of the case in the Patent Office.

Signed and sealed this 22nd day of January, A. D. 1952.

**[SEAL]**

**THOMAS F. MURPHY,  
Assistant Commissioner of Patents.**